

## UNITED STATES PATENT OFFICE

2,213,988

## LUBRICANT

Bert H. Lincoln, Ponca City, Okla., and Alfred Henriksen, deceased, late of Ponca City, Okla., by John W. Wolfe, administrator de bonis non, Ponca City, Okla., assignors, by mesne assignments, to The Lubri-Zol Development Corporation, Cleveland, Ohio, a corporation of Delaware

No Drawing. Application September 16, 1938,  
Serial No. 230,339

17 Claims. (Cl. 252—48)

Our invention relates to lubricating oils and particularly to an oil having high pressure-sustaining film-forming qualities.

This application is a continuation in part of copending application Serial No. 687,682, filed August 31, 1933.

Hydrocarbon lubricating oils per se will not withstand high pressures imposed during thin film or non-viscous lubrication. Under pressure the film of oil will rupture. A metal to metal contact under comparatively low loads results. This weakness, inherent in the very best quality hydrocarbon lubricants, has prevented designers of mechanical equipment from making certain desirable changes which would greatly improve mechanical devices in general.

One object of our invention is to increase the load-carrying properties of hydrocarbon lubricants by imparting to them an increased film strength.

Another object of this invention is to obtain such increased film strength without at the same time rendering the lubricating composition corrosive, especially to alloy bearing metals containing a characterizing proportion of cadmium, nickel, copper, lead, silver or tin and even to inhibit such corrosion by the lubricating oil base.

Other objects of this invention will appear as the description proceeds.

To the accomplishment of the foregoing and related ends, said invention, then, comprises the means hereinafter fully described and particularly pointed out in the claims, the following description setting forth in detail certain approved combinations of ingredients embodying my invention, such disclosed means constituting, however, but certain of various forms in which the principle of the invention may be used.

In general our invention comprises the addition of halogenated thioethers to hydrocarbon lubricants to obtain the desired film strength improvement.

It is believed that under conditions of extreme pressure the halogenated addition agents of this invention react chemically or physico-chemically with the metallic surfaces to form a non-fluxing surface which will not seize or score. This invention is not intended to be limited, however, by any particular theory or explanation of the action upon the metallic surfaces.

All of the various halogens are effective when employed in accordance with the present invention but chlorine is generally preferred inasmuch as it is the least expensive and one of the most effective of the halogens. Bromine and

fluorine are more expensive and the latter is relatively difficult to handle but they are each usable in accordance with this invention. Iodine is not so readily obtainable as the other halogens and is quite expensive but it also is satisfactory in providing effective addition agents. It should also be noted that two or more different halogens may be present in the same molecule. The bromo-chlor and fluorinated chlorine or bromine compounds give especially satisfactory results.

Halogenation may continue until sufficient halogen to form the mono-chlor product has been added or mixtures of less or greater halogen content may be employed. The halogen content of the halogenated thioether to be added to the lubricant may vary from about 5% to about 80%.

The halogenated thioethers contemplated for use in accordance with our invention will be found to be particularly useful in that they combine the desirable characteristics of both sulphur and halogen in a single addition agent and in such form that a cooperative result, not secured by any other type of addition agent, is attained. The outstanding characteristic of the halogenated thioethers which makes them particularly suitable as addition agents is their provision of generally higher film strength due to the combined presence of both sulphur and halogen in the oil, coupled with their corrosion inhibitor effect on the surfaces being lubricated. Unusually high film strength combined with effectiveness as a corrosion inhibitor is a characteristic not usually possessed by film strength addition agents.

Specific examples of the halogenated thioethers which may be employed in attaining the above-named desirable ends are as follows:

- (A) Chlorinated aliphatic thioethers: 40
  - (1) Dichloro-di-ethyl sulfide
  - (2) Chlorodi-n-butyl sulfide
  - (3) Chlorodilauryl sulfide
  - (4) Chloro-ethyl octadecyl sulfide
  - (5) Chloro-octadecyl butyl sulfide
- (B) Chlorinated aromatic thioethers: 50
  - (1) p,p'-Dichlorodiphenyl sulfide
  - (2) Trichlorodiphenyl sulfide
  - (3) o-Chlorophenyl naphthyl sulfide
  - (4) 2-chloronaphthyl phenyl sulfide
  - (5) 4,4'-Dinaphthyl sulfide
  - (6) Chlorodi (diphenyl) sulfide
  - (7) Monochloro-dibenzyl sulfide

- (C) Chlorinated mixed aromatic-aliphatic thio-ethers:
  - (1) p-Chloro-o-cresyl ethyl sulfide
  - (2) Chloroethyl phenyl sulfide
  - (3) 4-chloronaphthyl lauryl sulfide
  - (4) p-Nitro-o-chloro phenyl octadecyl sulfide
  - (5) 2-hydroxynaphthyl- $\beta$ -chloroethyl sulfide
  
- (D) Chlorinated alicyclic thio-ethers:
  - (1) Monochloro cyclohexyl sulfide
  - (2) Dichloro cyclohexyl sulfide
  - (3) Tetrachloro cyclohexyl sulfide
  - (4) Chloro cyclopentyl sulfide
  - (5) Chloro cyclobutyl sulfide
  - (6) Chloro methyl cyclohexyl sulfide
  - (7) Sym-dichlor dipentyl cyclohexyl sulfide
  - (8) Sym-dichlor dioctadecyl cyclohexyl sulfide
  - (9) Chloro cyclohexyl phenyl thio-ether
  - (10) Chloro cyclohexyl benzyl thio-ether
  
- (E) Chlorinated heterocyclic thio-ethers:
  - (1) Chloro furfuryl thio-ether
  - (2) Chloro furfuryl methyl thio-ether
  - (3) Chloro furfuryl phenyl thio-ether
  - (4) Chloro furfuryl cyclo hexyl thio-ether

25 Our invention is applicable to all classes of hydrocarbon lubricants, including hydrogenated lubricants, regardless of the S. A. E. classification or any other classification.

30 The base oil employed in the compositions of this invention is generally mineral oil, but it is to be understood that any other oil having suitable lubricating viscosity, whether naturally occurring or synthetic, and including hydrogenated oils, animal or vegetable oils such as castor oil, lard oil, corn oil, cottonseed oil and the like, may be employed as the oil base.

35 It is also within the contemplation of this invention to provide the addition agents in the form of a concentrate in a suitable oil, said oil containing rather high percentages of the addition agents. Such concentrates may be employed for future blending with a lubricating oil in the proportions desired for the particular conditions of use.

40 When used in conjunction with a mineral lubricating oil it is obvious that generally only such amounts of the addition agent may be included as are soluble in the specified amount of oil.

45 By the term "soluble" as herein used it is intended to indicate the ability to form not only true solutions but also any form of substantially permanently homogeneous composition when incorporated in mineral oil. With most of the compounds there is usually little difficulty, especially if the incorporation is effected in the manner described in Cornell Patent No. 2,042,880, and since quite small percentages often give remarkably improved results it is seldom of extreme importance that the addition agents be oil-soluble in all proportions.

50 The halogenated thioethers are quite effective when used in relatively small amounts as addition agents to lubricating compositions. This invention contemplates the use of from about 0.1% or even less to about 20% by weight, based on the amount of oil, of these addition agents and for the crankcase of internal combustion engines amounts from about 0.1% to about 2% are often sufficient. In the case of gear lubricants larger quantities, from about 2% to about 10%, may often be preferred. However, under certain relatively unusual circumstances where the thick-film and other properties of the ordinary mineral lubricating oil are not required to any great de-

gree the addition agent of this invention may be employed as the major component of the lubricating composition, only such proportion of lubricating oil being present as may be required to afford the characteristics desired.

5 Since, in general, the loss of the addition agent by volatilization will be less for compounds having a low volatility, the vapor pressure of the compounds should, for most purposes, be less than atmospheric pressure at temperatures up to 10 140° C. It is often desirable, especially for use in internal combustion engines, that the vapor pressure be less than atmospheric at temperatures up to 15 170° C. In the case of compounds which are stable at temperatures up to their boiling points, this condition may be expressed by stating that the boiling point of the compound should, in general, be higher than 140° C., and for certain uses, such as internal combustion engines, higher than 20 170° C.

25 While the lubricating compositions which have been described herein as illustrating one embodiment of the invention have been generally referred to as "oils," i. e., liquids, this invention is, however, also applicable to the solid and semi-solid types of lubricants commonly referred to in the trade as greases, bodied oils, etc.

30 The compounds of this invention are highly effective when employed as addition agents to lubricants for internal combustion engines such as airplane and Diesel engines. The halogenated thioethers are especially desirable for such uses inasmuch as both sulphur and halogen are found included in the same molecule thus affording a 35 very effective composition which is nevertheless safe and non-corrosive under difficult operating conditions.

40 While mineral oil generally is the principal ingredient of the lubricating composition, it is not essential that it be the only ingredient other than the addition agent, provided that there be no additional ingredient which is incompatible with such addition agent. It is within the contemplation of this invention to include, if necessary or desirable, such other addition agents as 45 are commonly added to improve the viscosity index or cold test of the lubricant and a lubricating composition according to this invention which also has a separate oiliness-increasing agent has been found to be especially effective.

50 Other modes of applying the principle of our invention may be employed instead of the one explained, change being made as regards the composition and method herein disclosed, provided the ingredients or steps stated by any of 55 the following claims or the equivalent of such stated ingredients or steps be employed.

We, therefore, particularly point out and distinctly claim as our invention:

1. A lubricating composition comprising a major proportion of mineral oil and a halogenated thio-ether.
2. A lubricant comprising in combination a major proportion of an oil of lubricating viscosity and a halogenated thio-ether.
3. A lubricating composition comprising a major proportion of mineral oil and a minor amount of a halogenated thio-ether.
4. A lubricating composition comprising a major proportion of mineral oil and from about 0.1% to about 20%, by weight based on the amount of mineral oil, of a halogenated thio-ether.
5. A lubricating composition comprising a major proportion of mineral oil and from about 0.1% 70 to about 20%, by weight based on the amount of mineral oil, of a halogenated thio-ether.

- to about 10%, by weight, based on the amount of mineral oil, of a halogenated thio-ether.
6. A lubricating composition comprising a major proportion of mineral oil and from about 0.1% to about 2%, by weight, based on the amount of mineral oil, of a halogenated thio-ether.
7. A lubricating composition comprising a major proportion of mineral oil and a minor amount of a halogenated thio-ether having a vapor pressure less than atmospheric at 140° C.
8. A lubricating composition comprising a major proportion of mineral oil and from about 0.1% to about 20%, by weight, based on the amount of mineral oil, of a halogenated thio-ether having a vapor pressure less than atmospheric at 140° C.
9. A lubricating composition comprising a major proportion of mineral oil and from about 0.1% to about 10%, by weight, based on the amount of mineral oil, of a halogenated thio-ether, having a vapor pressure less than atmospheric at 140° C.
10. A lubricating composition comprising a major proportion of mineral oil and from about 0.1% to about 2%, by weight, based on the amount of mineral oil, of a halogenated thio-ether having a vapor pressure less than atmospheric at 140° C.
11. A lubricating composition comprising a major proportion of mineral oil and a minor amount of a halogenated thio-ether having a vapor pressure less than atmospheric at 170° C.
12. A lubricating composition comprising a major proportion of mineral oil and from about 0.1% to about 20%, by weight, based on the amount of mineral oil, of a halogenated aliphatic thio-ether having a vapor pressure less than atmospheric at 140° C.
13. A lubricating composition comprising a major proportion of mineral oil and from about 0.1% to about 20%, by weight, based on the amount of mineral oil, of a halogenated aromatic thio-ether having a vapor pressure less than atmospheric at 140° C.
14. A lubricating composition comprising a major proportion of mineral oil and from about 0.1% to about 20%, by weight, based on the amount of mineral oil, of a halogenated alicyclic thio-ether having a vapor pressure less than atmospheric at 140° C.
15. A lubricating composition comprising a major proportion of mineral oil and from about 0.1% to about 20%, by weight, based on the amount of mineral oil, of a halogenated cyclic thio-ether having a vapor pressure less than atmospheric at 140° C.
16. A lubricating composition comprising a major proportion of mineral oil and from about 0.1% to about 20%, by weight, based on the amount of mineral oil, of a halogenated cyclo-aliphatic thio-ether having a vapor pressure less than atmospheric at 140° C.
17. A method of inhibiting scoring of relatively moving metallic surfaces under conditions of extreme pressure which comprises chemically-acting upon said surfaces with a halogenated thio-ether contained in a mineral oil.

BERT H. LINCOLN.

JOHN W. WOLFE,

*Administrator de bonis non of the Estate of  
Alfred Henriksen, Deceased.*

25

30

35

35